

# United States Patent [19]

Bourdoncle et al.

[11] 3,919,187

[45] Nov. 11, 1975

[54] **SULFUR-CONTAINING COMPOSITIONS OF UNSATURATED ESTERS, THEIR USE AS ADDITIVES FOR LUBRICANTS AND THE LUBRICATING COMPOSITIONS CONTAINING THEM**

[75] Inventors: **Bernard Bourdoncle**, Talance; **Bernard Sillion**, Grenoble, both of France

[73] Assignee: **Institut Francaise du Petrole, des Carburants et Lubrifiants, Rueil-Malmaison, France**

[22] Filed: **Oct. 29, 1973**

[21] Appl. No.: **410,531**

[30] **Foreign Application Priority Data**

Nov. 3, 1972 France ..... 72,39110  
Dec. 1, 1972 France ..... 72,42980

[52] **U.S. Cl.** ..... 260/125; 252/48.6

[51] **Int. Cl.<sup>2</sup>** ..... C10M 1/38; C07G 17/00

[58] **Field of Search** ..... 260/125; 252/48.6

[56] **References Cited**

UNITED STATES PATENTS

|           |         |               |         |
|-----------|---------|---------------|---------|
| 2,447,619 | 8/1948  | Rogers et al. | 260/125 |
| 2,454,862 | 11/1948 | Collins       | 260/125 |
| 2,569,122 | 9/1971  | Adelson       | 260/125 |
| 3,136,748 | 6/1964  | Miller et al. | 260/125 |
| 3,210,280 | 10/1965 | Rich          | 260/125 |

*Primary Examiner*—Lewis Gotts

*Assistant Examiner*—D. R. Phillips

*Attorney, Agent, or Firm*—Millen, Raptes & White

[57] **ABSTRACT**

Sulfurized compositions are obtained by sulfurizing an unsaturated ester obtained by esterifying at least one aliphatic mono- or di-carboxylic acid with at least one aliphatic ethylenically unsaturated mono-hydric alcohol. They are used as additives for mineral or synthetic oils.

**25 Claims, No Drawings**

**SULFUR-CONTAINING COMPOSITIONS OF UNSATURATED ESTERS, THEIR USE AS ADDITIVES FOR LUBRICANTS AND THE LUBRICATING COMPOSITIONS CONTAINING THEM**

The invention concerns new sulfur-containing compositions of unsaturated esters which may be used as additives for lubricants, and the lubricating compositions containing them.

It is known that the progress in the machine art tends towards still improved performances and therefore to the manufacture of more and more heavily loaded mechanisms, whose lubrication cannot be easily performed, particularly with respect to the persistence of the oil film, due to the existence of a limit running condition for lubrication. This is particularly true in the case of heavily loaded gears and also in the field of metal working, particularly metal cutting. When the persistence of the oil film can no longer be ensured, seizing occurs, which can result in the breaking of the machine or tool.

In order to avoid the above inconveniences, it has been proposed up to now to improve the lubricity of the oil, i.e. the resistance of the oil film, particularly by adding thereto a low proportion of sulfurized spermaceti oil. However, it is known that new regulations limit or forbid cachalot fishing so that natural spermaceti oil will be soon unavailable for industrial use at a reasonable price.

The invention has for object to provide new sulfurized compositions of unsaturated esters which can be used as additives for lubricants and are able to confer to mineral and synthetic lubricating oils lubricity, anti-wear and extreme-pressure properties at least equivalent to those obtained by means of sulfurized spermaceti oil.

Another object of the invention is to provide lubricity additives for lubricants, manufactured from starting materials which are easily available, cheap and not liable to become unavailable on the market.

The invention has for further object to provide lubricating compositions which have lubricity, anti-wear and extreme-pressure properties quite sufficient for satisfying the present requirements.

Generally speaking, the sulfurized compositions of the invention are obtained by sulfurizing ester compositions comprising a major proportion of one or more unsaturated esters formed by total esterification of:

- a. one or more saturated or unsaturated aliphatic mono- or di-carboxylic acids containing, for example, from 4 to 22 carbon atoms, with
- b. one or more ethylenically unsaturated aliphatic mono-hydric alcohols.

When considering the definition of the unsaturated esters of the invention, the aliphatic carboxylic acid may particularly consist of:

- a saturated chain monocarboxylic acid such as for example, 2-ethyl hexanoic acid, heptanoic acid, octanoic acid, nonanoic acid or iso-decanoic acid;
- a monocarboxylic acid having an unsaturated chain such as, for example, oleic acid (9-octadecenoic), linoleic acid (9,12-octadecadiene-oic) or undecenoic acid,
- or a mixture of saturated and unsaturated monocarboxylic acids, such as certain mixtures of fatty acids of animal origin, such as the fatty acids of tal-

low, or of vegetal origin, such as those obtained from soja-oil, colza-oil or by tall-oil distillation. The aliphatic carboxylic acid may also consist of: a dicarboxylic acid having a saturated straight chain, such as adipic acid, azelaic acid, sebacic acid or dodecane/dioic acid; or a dicarboxylic acid having a saturated branched chain such as, trimethyladipic acids or isononadecane/dioic acid,

or a dicarboxylic acid having an unsaturated straight chain, such as maleic or fumaric acid, or having an unsaturated branched-chain, such as alkenyl/succinic acid, for example tetrapropenyl/succinic acid.

The ethylenically unsaturated aliphatic monohydric alcohol usually comprises a straight or preferably branched aliphatic chain of at least 8 carbon atoms with at least one ethylenic unsaturation.

Among the aliphatic monohydric alcohols which can be used, we contemplate, according to a first embodiment of our invention, those which result from condensing formaldehyde with an aliphatic mono-olefin usually containing from 8 to 20 carbon atoms, thus containing, as a rule, from 9 to 21 carbon atoms.

In that case, the unsaturated aliphatic alcohol is preferably obtained from an aliphatic mono-olefin able to react with formaldehyde in the conditions of the Prins reaction with high yield. In this respect, it is advantageous to make use of an olefin having its ethylenic unsaturation at the end of the chain and linked to a completely substituted carbon atom.

Among the most suitable olefins, we can mention the following: isobutene dimer, propylene trimer, propylene tetramer, isobutene trimer and isobutene tetramer.

The condensation of formaldehyde on the olefin is usually carried out at a temperature of from 90° to 160°C, preferably in an autoclave, and in acetic, preferably anhydrous medium, for example during 6 to 20 hours. We preferably use for one mole of olefin:

from 0.8 to 1.5 mole of formaldehyde, preferably in the form of poloxymethylene, and from 100 to 350 ml of glacial acetic acid or a mixture of glacial acetic acid and acetic anhydride.

It may be advantageous to proceed at a moderate temperature of from 80° to 110°C, while using a catalyst, for example para-toluene/sulfonic acid or phosphoric acid, in a small amount, for example from 0.1 to 1% b.w. with respect to the reactants.

Conversely, it is preferable to avoid temperatures higher than 160°C, which would result in a cracking of the olefin and/or its condensation products to a certain extent, and also in the coloration of the reaction products.

The mixture obtained at the end of the reaction is distilled, optionally under vacuum, in order to remove the acetic solvent and, if necessary, all or part of the unreacted olefin fraction. This fraction, which may amount to 20-45 % of the olefin fed, may be recycled. The distillation residue is then washed with hot water, preferably alkali-containing water, so as to eliminate the residues of formaldehyde and acid, then saponified for example by means of an excess of sodium hydroxide dissolved in methanol. The saponification is carried out at reflux, for example for 0.5 to 2 hours, and is continued

until the product, after washing and drying, has a saponification number of approximately zero. This product will be referred to as "olefin condensation product".

Depending on the starting olefin, the olefin condensation product has a hydroxyl number, expressed in mg of potassium hydroxide per gram, of about 200 to 400 and an unsaturation degree, expressed as the number of ethylenic bonds per 100 g, of about 0.30-0.75. By way of illustration, Table I gives, for various starting olefins, the usual hydroxyl numbers and unsaturation degrees.

TABLE I

| Starting olefin    | Hydroxyl number<br>(mg KOH per gram) | Unsaturation<br>(= per 100 g) |
|--------------------|--------------------------------------|-------------------------------|
| Propylene trimer   | 330 - 370                            | 0.64 - 0.60                   |
| Propylene tetramer | 245 - 280                            | 0.51 - 0.48                   |
| Isobutene dimer    | 345 - 390                            | 0.70 - 0.66                   |
| Isobutene tetramer | 195 - 220                            | 0.39 - 0.36                   |

According to a second embodiment of the invention, the ethylenically unsaturated aliphatic alcohol is selected among those resulting from selectively reducing a branched  $\alpha,\beta$ -unsaturated aliphatic aldehyde, itself resulting from the aldolization-crotonization of one or more lower saturated aliphatic aldehydes of the formula:



where R is a straight alkyl radical and X is either a straight alkyl radical or a hydrogen atom, preferably a methyl radical or a hydrogen atom, and containing, for example, from 4 to 12 carbon atoms. The unsaturated aliphatic alcohol thus usually contains from 8 to 24 carbon atoms.

As examples of aldehydes of the general formula (I), which can be used as starting materials for the aldolization-crotonization reaction, the following may be mentioned:

n-butanal, n-pentanal, n-hexanal, n-heptanal, n-octanal, n-decanal, and the aldehydes obtained according to the "oxo" process from straight  $\alpha$ -olefins containing, for example, from 3 to 11 carbon atoms (the oxo process is well known: it consists of reacting, at high temperature and in the presence of a catalyst, a mixture of carbon monoxide and hydrogen with an olefin).

The latter aldehydes consist of mixtures of compounds of the formula (I) where X is a hydrogen atom or a methyl radical (in these mixtures, the straight aldehydes are in major proportion, usually about 75 %).

The aldolization-crotonization of aldehydes is also well-known. It is disclosed, for example, in *Organic Reactions*, John Wiley and Sons, New York (1968), volume 16. It consists in condensing an aldehyde on itself or on another aldehyde, usually in the presence of a basic catalyst, and dehydrating the alcohol formed.

By aldolization-crotonization of the saturated aldehydes of the formula (I) above, there are obtained branched  $\alpha,\beta$ -unsaturated aliphatic aldehydes (containing, for example, from 8 to 24 carbon atoms), from which are obtained, by selective reduction, the unsaturated alcohols employed for preparing the unsaturated esters of the invention.

The selective reduction of these  $\alpha,\beta$ -unsaturated aldehydes to unsaturated alcohols may be achieved according to any conventional method. It is thus possible to make use of a reducing compound such as, for example, aluminium-lithium hydride, aluminium iso-propox-

ide, potassium or sodium borohydride. However, for economic reasons, molecular hydrogen is preferably employed, in the presence of a convenient catalyst, such as, for example, partially poisoned platinum oxide, partially poisoned platinum-on-carbon, lead-inhibited ruthenium or osmium or a carbon or alumina carrier, the latter two catalysts giving the best results.

The catalytic reduction with hydrogen may be carried under relatively mild conditions, for example at a temperature of about 80°-160°C under a hydrogen pressure of about 30-120 kg/cm<sup>2</sup>. Preferably we proceed in an autoclave provided with an efficient stirring system. At the end of the reaction, the catalyst is separated and recovered for example, by filtration. It must be noted that a solvent is not necessary, as far as the reduction of the  $\alpha,\beta$ -unsaturated aldehydes used according to the invention is concerned, although it may facilitate filtering of the reaction product and consequently recovering the catalyst. There is used, for example, an alcohol such as isopropanol. After the filtering of the reaction product and an optional vaporization of the solvent, there is obtained an unsaturated alcohol or a mixture of unsaturated alcohols which can be used for manufacturing the compositions of unsaturated esters according to the invention.

Depending on the starting saturated aldehyde (or mixture of aldehydes), the resulting unsaturated alcohol (or mixture of alcohols) has a variable hydroxyl number (for example about 16 to 44 milligrams of potassium hydroxide per gram of product) and a variable unsaturation degree (for example about 0.28 to 0.76 ethylenic double bond per 100 g of product).

The total esterification of the aliphatic carboxylic acid or acid mixture with the unsaturated aliphatic monohydric alcohol may be carried out according to any convenient method.

For example, we may proceed at reflux of a solvent such as, for example, benzene, toluene or a xylene, with azeotropic removal of the formed water, and catalyze the reaction by means of a small amount, for example 0.1-2% b.w., of an acid such as para-toluene/sulfonic acid. After evaporation of the solvent, the esterification product may be purified, for example by passing it on activated earth.

According to other ways of manufacturing the unsaturated ester compositions, we may use, instead of the mono- and di-carboxylic acids themselves, some of their functional derivatives, such as their halides (for example their chlorides), anhydrides or lower alkyl esters.

When preparing compositions of unsaturated esters, without departing from the invention, the ethylenically unsaturated aliphatic mono-hydric alcohol(s) may be used in admixture with a minor proportion of one or more saturated aliphatic alcohols, particularly for adjusting the unsaturation degree of the feeding mixture of alcohols to be subjected to esterification and consequently the unsaturation degree of the ester compositions resulting therefrom. These saturated aliphatic alcohols, which contain, for example, from 6 to 20 carbon atoms, may consist of alcohols having a saturated aliphatic straight chain, such as, for example, hexanol, heptanol, octanol, nonanol, decanol, dodecanol or eicosanol, or of alcohols having a saturated aliphatic branched chain such as, for example, 2-ethyl hexanol or alcohols obtained by oxo synthesis from olefins, for example iso-nonanol, iso-decanol and iso-tridecanol.

They can be used in a proportion of from 10 to 30 % by weight of the total weight of the alcohols subjected to esterification, depending on the desired unsaturation degree of the resulting ester composition.

The sulfur-containing compositions of the invention result from the sulfurization of ester compositions such as hereinbefore described, particularly those having an unsaturation degree of from about 0.20 to about 0.55 ethylenic bond per 100 grams.

These compositions may be sulfurized, for example up to a content of about 6 to 15 % by weight of sulfur, depending on the case, according to any convenient technique. For example, the following technique may be used:

From 7 to 20 parts b.w. of elemental sulfur and from 0.5 to 2 parts b.w. of zinc oxide are added to 100 parts b.w. of an ester composition, such as hereinbefore defined. The stirred mixture is heated in a first step at a temperature of from 145° to 175°C, for example for 5-10 hours, in an inert atmosphere. After this first treatment, the temperature is raised in a second step to 180°-188°C, for example during 2-4 hours. During this second step, a minor proportion of the fixed sulfur, for example about 10 % of the total sulfur content of the charge, is removed in the form of hydrogen sulfide. There is thus obtained, after filtering, a sulfurized product according to the invention.

The following technique may also be used:

7-20 parts by weight of elemental sulfur and 0.5-4 parts b.w. of a secondary aliphatic amine, for example dicyclohexylamine, are added to 100 parts by weight of the ester composition. The stirred mixture is heated at a temperature of from 130° to 160°C, for example during 5-10 hours, under an atmosphere which is inert with respect to the reactants. After filtering, the sulfurized product of the invention is obtained.

It may be advantageous to conduct the sulfurization reaction, for example, according to one of the hereinbefore described methods, with an ester composition diluted with a minor proportion, for example 10-40 % b.w., of a substrate such as a light mineral oil, corresponding for example to the SAE grade 10 W or 5 W or a synthetic oil, for example iso-decyl adipate or 2-ethyl hexyl maleate.

Finally, if the extreme-pressure properties of the obtained sulfurized product are to be specifically enhanced, it is convenient to have it react, for example for 2-8 hours at a temperature of 90°-120°C, with a lower proportion, for example 0.2-0.6 % by weight of phosphorus sesquisulfide ( $P_4S_3$ ).

The sulfurized products of the invention are used as additives for lubricants, either for mineral oils or for synthetic oils. As a rule, they are added to the lubricating bases in an amount of from 0.5 to 10 % by weight and preferably from 1 to 5 % by weight of the lubricating base. They confer to the latter base very substan-

tially improved anti-wear and extreme-pressure properties, without noticeably modifying the pour point. The resulting lubricating compositions also have an extremely low corrosivity with respect to usual metals, particularly copper.

The following examples illustrate the invention and must not be considered as limitative thereof. The unsaturation numbers given in these examples have been determined by the Brown method consisting of a selective catalytic hydrogenation of the ethylenic bonds on palladium.

#### EXAMPLE I

252.5 g (2 moles) of propylene trimer, 72 g (2.4 moles) of paraformaldehyde and 500 ml of glacial acetic acid are introduced into a stirred autoclave. The mixture is heated at 120°C for 10 hours and strongly stirred. Acetic acid and a portion (about 95 g) of the unreacted olefin are separated by distillation. The residue is washed with hot water (80°C) and then treated at 100°C with a 10 N solution of sodium hydroxide in a mixture of water and methanol. After careful washing with water, there are recovered 205 g of olefin condensation product in the form of an oily liquid of straw yellow colour, having the following characteristics:

Hydroxyl number 341 mg of potassium hydroxide per gram.

Unsaturation: 0.62 ethylenic bond per 100 g.

164 g (one hydroxyl equivalent) of this olefin condensation product, 282 g (1 mole) of oleic acid, 2 g of paratoluene/sulfonic acid and 150 ml of benzene are poured into a 2 liter flask. The mixture is heated at smooth reflux. Any formed water is continuously collected by decantation in a Dean and Stark apparatus. During esterification, temperature remains at 120°-130°C. After 9 hours, 17.6 g of water collected and heating is discontinued. After water-washing and benzene-evaporating, 425 g of unsaturated ester composition ester composition are obtained.

200 g of this unsaturated ester composition, 26 g of sulfur and 2 g of zinc oxide are introduced into a 500 ml reactor provided with stirring means. The mixture is heated and stirred under nitrogen for 7 hours at 160°C, then 3 hours at 180°C. After filtering, 222 g of Additive

30 I are obtained, said additive having the following characteristics:

viscosity at 98.9°C: 21 cst

pour point: -15°C

sulfur content 10.8 % by weight

#### EXAMPLES 2-6

Various olefin condensation products have been prepared according to the technique of Example 1.

The nature and amounts of reactants, as well as the nature and characteristics of the obtained condensation products are summarized in Table II below:

TABLE II

| Ex. | Nature    | Olefin     |         | Para             |       |            | Olefin condensation product |                 |  |
|-----|-----------|------------|---------|------------------|-------|------------|-----------------------------|-----------------|--|
|     |           | Amount (g) | (moles) | formaldehyde (g) | (mls) | weight (g) | hydroxyl number(1)          | unsaturation(2) |  |
| 2   | isobutene |            |         |                  |       |            |                             |                 |  |
|     | dimer     | 448.8      | 4       | 144              | 4.8   | 396        | 362                         | 0.68            |  |
| 3   | propylene | 673        | 4       | 144              | 4.8   | 558        | 255                         | 0.49            |  |
|     | tetramer  |            |         |                  |       |            |                             |                 |  |
| 4   |           |            |         |                  |       |            | as in Example 3             |                 |  |
| 5   |           |            |         |                  |       |            | as in Example 3             |                 |  |
| 6   |           |            |         |                  |       |            | as in Example 1             |                 |  |

(1) in mg of potassium hydroxide per gram

(2) in number of ethylenic bonds per 100 grams

According to the same technique as in Example 1, each of the so obtained olefin condensation products is used to esterify a carboxylic acid, in order to form the corresponding unsaturated ester compositions. The nature and amounts of reactants, as well as the obtained amount of unsaturated ester composition are indicated in Table III below:

b.w. (11.5 g) of a 5 % osmium catalyst on an alumina carrier. The temperature is raised to 100°C, the hydrogen pressure to 70 kg/cm<sup>2</sup> and the stirring started.

When no more hydrogen absorption is observed, the reaction mixture is cooled, diluted with 250 ml of isopropanol and filtered, in order to separate the catalyst therefrom. After vaporization of iso-propanol, 231 g of

TABLE III

| Ex. | Conden. Prod. weight | Eq.OH | Nature          | Saturated alcohol amount (g) eq.OH |      | nature                | Carboxylic acid amount g. | acid eq. | Ester (g) |
|-----|----------------------|-------|-----------------|------------------------------------|------|-----------------------|---------------------------|----------|-----------|
|     |                      |       |                 | 65                                 | 0.5  |                       |                           |          |           |
| 2   | 232                  | 1.5   | 2-ethyl hexanol | 65                                 | 0.5  | adipic acid           | 146                       | 2        | 403       |
| 3   | 440                  | 2     | none            | none                               | none | adipic acid           | 146                       | 2        | 546       |
| 4   | 440                  | 2     | none            | none                               | none | oleic ac.             | 282                       | 1        |           |
| 5   | 165                  | 0.75  | isononanol      | 36                                 | 0.25 | maleic an.            | 49                        | 1        | 741       |
| 6   | 164                  | 1     | none            | none                               | none | fatty ac. of Tall-oil | 288                       | 1        | 484       |
|     |                      |       |                 |                                    |      | dodecanoic acid       | 115                       | 1        | 258       |

200 g of each of the so obtained unsaturated ester compositions have been sulfurized in the conditions of Example 1. Table IV gives the proportions of employed sulfur and zinc oxide, the amount of obtained sulfurized product and the characteristics thereof.

TABLE IV

| Ex. | S (g) | ZnO (g) | Name     | Obtained sulfurized product |                        |                 |      | %S b.w. |
|-----|-------|---------|----------|-----------------------------|------------------------|-----------------|------|---------|
|     |       |         |          | weight (g)                  | viscosity 98.9°C (cSt) | pour point (°C) |      |         |
| 2   | 28    | 2       | Add. II  | 224                         | 30                     | -21             | 12.3 |         |
| 3   | 23    | 2       | Add. III | 219                         | 24                     | -17             | 9.1  |         |
| 4   | 18    | 2       | Add. IV  | 214                         | 29                     | -12             | 7.5  |         |
| 5   | 37    | 2       | Add. V   | 229                         | 37                     | -9.5            | 14.1 |         |
| 6   | 25    | 2       | Add. VI  | 221                         | 34                     | -14             | 10.0 |         |

## EXAMPLE 7

a. 75 ml of a 1 N sodium hydroxide solution in water are heated at 80°C in a 500 ml reaction vessel provided with a mechanical stirrer, a bulb cooler maintained at 5°C and a 350 ml bromine funnel. 252 g of n-heptanal are introduced dropwise in 1 h 30 mn through the bromine funnel. After heptanal addition, the temperature is raised so as to obtain a gentle reflux, which is maintained for 1 h 30 mn. The reaction mixture is then cooled and carefully washed with water, in the presence of hexane, up to neutrality. After hexane evaporation, 230 g of  $\alpha,\beta$ -unsaturated C<sub>14</sub> aldehyde are obtained.

The so obtained  $\alpha,\beta$ -unsaturated aldehyde is placed in a 500 ml stirred autoclave, in the presence of 5 %

unsaturated alcohol are collected, said alcohol having the following characteristics:

Hydroxyl number: 264 mg KOH per gram

Unsaturation number: 0.47 = per 100 g.

b. 212 g (1 hydroxyl equivalent) of this unsaturated alcohol, 73 g (1 acid equivalent) of adipic acid, 1 g of para-toluene/sulfonic acid and 100 ml of benzene are introduced into an 1 liter flask. The mixture is heated at gentle reflux. The formed water is continuously collected by decantation in a Dean and Stark system. During the esterification, the temperature remains at 120°-130°C. After 8 hours, 17.8 g of water have been collected and heating is discontinued. After water-washing and benzene-vaporizing, 265 g of unsaturated ester are obtained, said ester having an unsaturation number of 0.37 = per 100 g.

c. 200 g of this unsaturated ester, 25 g of sulfur and 4 g of dicyclohexylamine are introduced into a 500 ml reactor provided with a mechanical stirrer. The mixture is heated and stirred under nitrogen at 155°C for 6 hours. 223 g of Additive VII are obtained, said Additive being so characterized:

Viscosity at 98.9°C: 32 cSt

Pour point: -14°C

Sulfur content: 10.6 % b.w.

## EXAMPLES 8-14

a. According to the same technique as in Example 7(a), various  $\alpha,\beta$ -unsaturated aliphatic aldehydes and the corresponding unsaturated alcohols have been prepared.

The nature and amounts of reactants and intermediary products, and the amounts and characteristics of the obtained unsaturated alcohols are summarized in Table V below:

TABLE V

| Ex.  | Saturated aldehyde                             |            | $\alpha,\beta$ -unsaturated aldehyde |            | OH number (4) | unsaturation (5) |
|------|------------------------------------------------|------------|--------------------------------------|------------|---------------|------------------|
|      | nature                                         | amount (g) | nature                               | amount (g) |               |                  |
| 8a)  |                                                |            | Example 7 a)                         |            |               |                  |
| 9a)  |                                                |            | as Example 7 a)                      |            |               |                  |
| 10a) | n-butanal <sup>(1)</sup>                       | 252        | C <sub>8</sub>                       | 216        | 437           | 0.74             |
| 11a) | C <sub>6</sub> -C <sub>8</sub> <sup>(2)</sup>  | 252        | C <sub>12</sub> -C <sub>16</sub>     | 232        | 258           | 0.42             |
| 12a) | mixture                                        | 252        | as Example 11 a)                     |            |               |                  |
| 13a) | C <sub>8</sub> -C <sub>10</sub> <sup>(3)</sup> | 252        | C <sub>18</sub> -C <sub>20</sub>     | 143        | 200           | 0.35             |
| 14a) |                                                |            | as Example 7 a)                      |            |               |                  |

<sup>(1)</sup>During n-butanal addition, the temperature must not exceed 90°C. After complete introduction of n-butanal, the vessel is heated under gentle reflux.

<sup>(2)</sup>The mixture, obtained from a cut of straight  $\alpha$ -olefins C<sub>8</sub> - C<sub>7</sub> by oxo-reaction, contains by mole: n-hexanal + 2-methyl pentanal: 20%; n-heptanal + 2-methyl hexanal: 50%; n-octanal + 2-methyl heptanal: 30%.

<sup>(3)</sup>The mixture, obtained from a cut of straight  $\alpha$ -olefins C<sub>8</sub> - C<sub>9</sub> by oxo-reaction, contains by mole: n-nonanal + 2-methyl octanal: 30%; n-decanal + 2-methyl nonanal: 70%.

<sup>(4)</sup>The hydroxyl number is expressed in mg of potassium hydroxide per gram of product.

<sup>(5)</sup>The unsaturation number is expressed as the number of ethylenic double bonds per 100 g of product.

b. According to the same technique as in Example 7(b), each of the so-obtained unsaturated alcohols is used to esterify a carboxylic acid to form the corresponding unsaturated esters. The nature and amounts of reactants and also the amount of obtained unsaturated ester are given in Table VI:

TABLE VI

| Ex.  | unsat.alcohol |        | nature                                      | saturated alc. |          | nature                              | carboxylic acid |          | ester |          |
|------|---------------|--------|---------------------------------------------|----------------|----------|-------------------------------------|-----------------|----------|-------|----------|
|      | weight (g)    | OH Eq. |                                             | amount (g)     | (OH Eq.) |                                     | amount (g)      | acid eq. | (g)   | Uns. (2) |
| 8b)  | 212           | 1      | none                                        | none           | none     | dodeca-nedioic oleic                | 115             | 1        | 307   | 0.32     |
| 9b)  | 148.4         | 0.7    | 2-ethyl hexanol                             | 39             | 0.3      |                                     | 282             | 1        | 450   | 0.32     |
| 10b) | 128           | 1      | none                                        | none           | none     | isonona-decane-dioic azelaic adipic | 164             | 1        | 271   | 0.34     |
| 11b) | 217           | 1      | none                                        | none           | none     |                                     | 94              | 1        | 291   | 0.31     |
| 12b) | 173.6         | 0.8    | n-heptanol                                  | 23.2           | 0.2      |                                     | 73              | 1        | 250   | 0.29     |
| 13b) | 196           | 0.7    | mixture C <sub>8</sub> -C <sub>10</sub> (1) | 39.9           | 0.3      | Tall oil fatty acids                | 288             | 1        | 520   | 0.41     |
| 14b) | 212           | 1      | none                                        | none           | none     | nonanoic                            | 158.2           | 1        | 351   | 0.26     |

(1)The mixture, whose hydroxyl number is 421 mg of KOH/g, contains by mole: n-hexanol: 21%; n-octanol: 35%; n-decanol: 44%

(2)The unsaturation number is expressed as the number of ethylenic double bonds per 100 g of product.

c. 200 g of each of the so-obtained unsaturated esters have been sulfurized in the conditions of Example 7(c). Following Table VII gives: the amounts of employed sulfur and dicyclohexylamine, the amount of obtained sulfurized product and the characteristics thereof.

TABLE VII

| Ex.  | S (g) | Di-cyclohexyl-amine (g) | name        | Resulting sulfurized product |                    |                 |      | % S b.w. |
|------|-------|-------------------------|-------------|------------------------------|--------------------|-----------------|------|----------|
|      |       |                         |             | wt. (g)                      | visco-98.9°C (cSt) | pour point (°C) | b.w. |          |
| 8c)  | 22    | 4                       | Addit.VIII  | 219                          | 37                 | -12             | 8.9  |          |
| 9c)  | 35    | 4                       | Addit.IX    | 232                          | 41                 | -11             | 13.9 |          |
| 10c) | 28    | 4                       | Addit. X    | 225                          | 39                 | -16             | 11.2 |          |
| 11c) | 18    | 4                       | Addit. XI   | 216                          | 29                 | -16             | 7.4  |          |
| 12c) | 27    | 4                       | Addit. XII  | 223                          | 35                 | -18             | 10.9 |          |
| 13c) | 26    | 4                       | Addit. XIII | 224                          | 38                 | -7              | 10.8 |          |
| 14c) | 23    | 4                       | Addit.XIV   | 220                          | 22                 | -9              | 9.0  |          |

10  
In order to evaluate the anti-wear and extreme-pressure qualities of the products obtained according to Examples 1-14, each of them has been dissolved in a proportion of 3 % b.w. in a base oil (A) and the resulting compositions have been tested with test machines.

Base oil (A) is a mixture by equal parts of 150 neutral mineral oil and a 450 Neutral mineral oil.

The test machines are, on the one hand, the four-balls machine (E.P.Tester) for determining the Load-Wear Index (L.W.I.) according to ASTM standard D-2783-71 and, on the other hand, the machine FZG for determining the damage level (i.e. the seizing level noted from 1 to 12) and the specific wear (i.e. the average slope of the wear curve before seizing, expressed in mg/horse power-hour) according to the German standard DIN 51 354 of January 1970, with gear weighing.

Table VIII gives the results obtained with compositions containing Additives I to XIV. By way of comparison, there are given the results obtained with base oil (A) alone and with the same base oil containing 3 % by weight of sulfurized spermaceti oil.

TABLE VIII

| Composition                               | L.W.I. (kg) | Damage level | Specific wear mg/Ch.h |
|-------------------------------------------|-------------|--------------|-----------------------|
| Base oil (A)                              | 20.1        | 6            | 0.320                 |
| (A)+30% b.w. of sulfurized spermaceti oil | 45.2        | 10           | 0.142                 |
| (A) + 3% b.w. of Additive I               | 60.7        | 11           | 0.116                 |
| (A) + 3% b.w. of Additive II              | 58.9        | 12           | 0.109                 |
| (A) + 3% b.w. of Additive III             | 54.0        | 10           | 0.112                 |

55  
(A) + 3% b.w. of Additive IV 53.2 10 0.122  
(A) + 3% b.w. of Additive V 63.1 12 0.117  
(A) + 3% b.w. of Additive VI 60.0 11 0.109  
(A) + 3% b.w. of Additive VII 57.2 11 0.135  
(A) + 3% b.w. of Additive VIII 56.8 10 0.132  
(A) + 3% b.w. of Additive IX 58.0 11 0.129  
(A) + 3% b.w. of Additive X 60.1 12 0.121  
(A) + 3% b.w. of Additive XI 56.5 10 0.130  
(A) + 3% b.w. of Additive XII 59.3 12 0.091  
(A) + 3% b.w. of Additive XIII 58.7 11 0.114  
(A) + 3% b.w. of Additive XIV 56.6 10 0.133

60  
The improvement of the anti-wear and extreme-pressure properties of the oil, resulting from the addition of the sulfurized products of the invention, is quite remarkable. It is substantially better than when using sulfurized spermaceti oil.

What we claim is:

1. A sulfur-containing composition obtained by sulfurizing an ester composition having a degree of unsatu-

## 11

ration of 0.20-0.55 double bonds per 100 grams, said ester being formed by total esterification of:

- a. at least one aliphatic hydrocarbyl mono- or di-carboxylic acid means with
  - b. at least one aliphatic hydrocarbyl monohydric alcohol means consisting essentially of 70-100% by weight of at least one branched aliphatic hydrocarbyl unsaturated monohydric alcohol having about 1 ethylenic unsaturation and containing at least 8 carbon atoms and 0-30% by weight of at least one saturated aliphatic hydrocarbyl monohydric alcohol.
2. A composition according to claim 1, wherein the mono- or di-carboxylic acid means contains 4-22 carbon atoms.
3. A composition according to claim 1, wherein said monohydric alcohol means consists essentially of about 100% of the branched unsaturated alcohol.
4. A composition according to claim 1, wherein the ester composition results from totally esterifying:

- a. at least one aliphatic hydrocarbyl mono- or dicarboxylic acid means with
- b. 70-90% by weight of the at least one branched aliphatic hydrocarbyl unsaturated monohydric alcohol and 10-30% by weight of the at least one saturated aliphatic hydrocarbyl monohydric alcohol.

5. A composition according to claim 1, wherein the saturated aliphatic monohydric alcohol contains from 6 to 20 carbon atoms.

6. A composition according to claim 1, wherein the aliphatic mono- or di-carboxylic acid means comprises a halide, an anhydride or a lower alkyl ester.

7. A composition according to claim 1, wherein the sulfurization degree is 6-15% by weight of sulfur.

8. A composition according to claim 7, wherein the sulfurization is carried out by heating the ester composition in the presence of a convenient amount of elemental sulfur, so as to obtain the desired sulfurization degree and the obtained product is filtered.

9. A composition according to claim 1, wherein the sulfurization is carried out on the ester composition previously diluted in a diluent comprising isodecyl adipate or 2-ethylhexyl maleate.

10. A composition according to claim 9, wherein the diluent amounts to 10-40% by weight of the ester composition.

11. A composition according to claim 1, wherein the ethylenically, unsaturated aliphatic monohydric alcohol results from condensing formaldehyde with a branched monoolefin of 8-20 carbon atoms, said alcohol itself containing 9-21 carbon atoms.

12. A composition according to claim 11, wherein the branched aliphatic monoolefin is isobutene dimer, propylene trimer, propylene tetramer, isobutene trimer or isobutene tetramer.

13. A composition according to claim 1, wherein the aliphatic hydrocarbyl ethylenically unsaturated monohydric alcohol contains 8-24 carbon atoms and results from selectively reducing a branched  $\alpha,\beta$ -unsaturated aliphatic aldehyde, itself resulting from the aldolization-crotonization of at least one saturated aliphatic aldehyde of 4-12 carbon atoms and of the general formula:



## 12

in which R is a straight alkyl radical and X is selected from the hydrogen atom and the straight alkyl radicals.

14. A composition according to claim 13, wherein X is a hydrogen atom or a methyl radical in the formula of the saturated aliphatic aldehyde.

15. A composition according to claim 7, wherein the monohydric alcohol means consists essentially of about 100% of the at least one unsaturated alcohol.

16. A composition according to claim 7, wherein the ester composition results from the complete esterification of:

- a. At least one aliphatic hydrocarbyl mono- or dicarboxylic acid means with
- b. 70-90% by weight of the at least one aliphatic hydrocarbyl ethylenically unsaturated monohydric alcohol and 10-30% by weight of the at least one saturated aliphatic hydrocarbyl monohydric alcohol.

17. A composition according to claim 16, wherein the saturated aliphatic monohydric alcohol contains from 6 to 20 carbon atoms.

18. A composition according to claim 17, wherein the aliphatic mono- or di-carboxylic acid means comprises a halide, an anhydride or a lower alkyl ester.

19. A composition according to claim 3, wherein the sulfurization degree is 6-15% by weight of sulfur.

20. A composition according to claim 19, wherein the sulfurization is carried out by heating the ester composition in the presence of a convenient amount of elemental sulfur, so as to obtain the desired sulfurization degree and the obtained product is filtered.

21. A composition according to claim 20, wherein the sulfurization is carried out on the ester composition previously diluted in a diluent comprising isodecyl adipate or 2-ethylhexyl maleate.

22. A composition according to claim 7, wherein the ethylenically unsaturated aliphatic monohydric alcohol results from condensing formaldehyde with a branched aliphatic mono-olefin of 8-20 carbon atoms, said alcohol itself containing 9-21 carbon atoms.

23. A composition according to claim 22, wherein the branched aliphatic monoolefin is isobutene dimer, propylene trimer, propylene tetramer, isobutene trimer or isobutene tetramer.

24. A composition according to claim 20, wherein the aliphatic hydrocarbyl ethylenically unsaturated monohydric alcohol contains 4-8 carbon atoms and results from selectively reducing a branched  $\alpha,\beta$ -unsaturated aliphatic aldehyde, itself resulting from the aldolization-crotonization of at least one saturated aliphatic aldehyde of 4-12 carbon atoms and of the general formula:



in which R is a straight alkyl radical and X is selected from the hydrogen atom and the straight alkyl radicals.

25. A composition according to claim 24, wherein X is a hydrogen atom or a methyl radical in the formula of the saturated aliphatic aldehyde.

\* \* \* \* \*